

1

3,255,078

PROCESS FOR THE TREATMENT OF FIBER ARTICLES OF SYNTHETIC POLYAMIDES AND COMPOSITION PRODUCED

Karl-August Heinroth and Robert Schnegg, Dormagen, Fritz Steinfatt, Opladen, and Christian Wiegand, Elberfeld, Germany, assignors to Farbenfabriken Bayer Aktiengesellschaft, Leverkusen, Germany, a German corporation

No Drawing. Filed July 13, 1961, Ser. No. 123,623  
Claims priority, application Germany, July 23, 1960,

31,754

3 Claims. (Cl. 167—38.6)

The present invention relates to the treatment of fiber articles of synthetic polyamides; more particularly it concerns a process for the treatment of fiber articles of synthetic polyamides which consists in treating the fiber articles with antimicrobial arylene imidazolium compounds.

In this way it is possible to finish fiber articles of synthetic polyamides such as fibers, filaments, yarns, fabrics as well as wearing apparel made therefrom, in an outstanding antimicrobial manner. Surprisingly, this finish is very fast to washing such as is required for fiber articles of synthetic polyamides. Furthermore, it is noteworthy that the textile materials treated according to the invention have a strongly deodorizing and anti-perspiration effect.

The treatment of the fiber articles is advantageously carried out in an aqueous medium and at an elevated temperature. Suitable antimicrobial arylene imidazolium compounds have been described, for example, in French patent specification No. 1,248,412; they correspond to the general formula



In this formula X represents an acid radical, for example the radical of hydrochloric acid, sulfuric acid or methylsulfuric acid or a radical of a phosphoric acid or a low molecular weight aliphatic carboxylic acid, Y stands for an aryl radical, for instance for a phenyl or naphthyl radical which may be substituted, for example by halogen and/or hydroxyl groups, or for a heterocyclic radical, for example the furyl, pyrrol, thieryl, pyridyl, indolyl or quinolyl radical; one of the substituents R<sub>1</sub> and R<sub>2</sub> is an alkyl radical or an esterified or amidated acid group which contains 1-4 carbon atoms and the other substituent is an alkyl radical or an esterified or amidated acid group which contains at least 10 carbon atoms.

Suitable quantities of the arylene imidazolium compounds may easily be determined by preliminary experiments; in general, it is advisable to use the compounds in the form of 0.2-5% aqueous solutions.

The following examples serve to illustrate the invention without, however, limiting the scope thereof.

*Example 1*

A knitted fabric of spun-dyed filaments produced from commercial synthetic polyamides is agitated at 95° C. for 60 minutes in an aqueous solution using a goods-to-liquor ratio of 1:40 and containing, per liter, 2 g. of

2

1-methyl-2-phenyl-3-dodecyl-benzimidazolium bromide. The fabric is subsequently rinsed and then dried.

The textile material thus treated has an antimicrobial finish. The outstanding fastness to washing of this finish can be seen in the following table in which the width of the inhibition zones which result around samples of the finished textile material placed on agar-agar plates inoculated with the various microbes given in the table before washing and after washing several times with a commercial detergent, is indicated in millimeters.

Table

|                            | <i>Stc. aureus</i> | <i>Bct. fluoresc.</i> | <i>Trichop. mentagroph.</i> |
|----------------------------|--------------------|-----------------------|-----------------------------|
| Before washing.....        | 3                  | 3                     | 5                           |
| After washing once.....    | 3                  | 3                     | 4                           |
| After washing 5 times..... | 3                  | 3                     | 3                           |

*Example 2*

A fabric produced from undyed filaments of polymeric  $\epsilon$ -caprolactum is agitated for 2 hours in an aqueous bath which contains, per liter, 20 g. of 1-methyl-2-phenyl-3-dodecyl-benzimidazolium bromide; the initial temperature of 40° C. is slowly raised to 98° C. The fabric is then rinsed, and dried at 80-100° C. for some minutes.

Testing of the fabric thus treated as to its antimicrobial effect in the plate test described in Example 1 gave the following values for the width of the inhibition zones in millimeters:

|                             |   |
|-----------------------------|---|
| <i>Stc. aureus</i> .....    | 3 |
| <i>Bct. fluoresc.</i> ..... | 2 |
| <i>Trichop. ment.</i> ..... | 4 |
| <i>Candida alb.</i> .....   | 4 |

*Example 3*

Socks produced from filaments of polymeric  $\epsilon$ -caprolactam are agitated for 60 minutes in an aqueous bath having a goods-to-liquor ratio of 1:40 and containing, per liter, 50 g. of 1-methyl-2-phenyl-3-dodecyl-benzimidazolium bromide, the initial temperature of 40° C. being slowly raised to 98° C. The socks are finally dried. Their antimicrobial finish was also found to be very fast to washing.

The outstanding suitability of the antimicrobial arylene imidazolium compounds to be used according to the invention is surprising since other known, highly active antimicrobial agents, such as quaternary ammonium compounds of the dimethyl-dodecyl-benzyl-ammonium chloride type, or halogenated dihydroxy-diphenyl compounds of the dichloro-dihydroxy-diphenyl methane type, do not yield satisfactory results in the treatment of fiber articles of synthetic polyamides.

The term "synthetic polyamides" herein used denotes long-chain synthetic polyamides which have recurring amide groups as an integral part of the main polymer chain and which are capable of being formed into filaments; such synthetic polyamides may be derived from hexamethylene diamine and adipic acid, from  $\epsilon$ -aminocaproic acid or from  $\epsilon$ -caprolactam (cf. Kirk-Othmer: "Encyclopedia of Chemical Technology," vol. 10, New York, 1953, pages 916-917).

We claim:

1. Process for imparting antimicrobial properties to fiber articles of long-chain synthetic polyamides having

3

recurring amide groups as an integral part of the main polymer chain, comprising contacting the articles in an aqueous medium with an active amount of 1-methyl-2-phenyl-3-dodecyl-benzimidazolium bromide.

2. A method for imparting antimicrobial properties to fiber articles of long-chain synthetic polyamides having recurring amide groups as an integral part of the main polymer chain, comprising contacting the fiber articles with an active amount of a compound having the formula



wherein X is an acid anion; Y is phenyl; R<sub>1</sub> is an alkyl of 1-4 carbon atoms; and R<sub>2</sub> is an alkyl which contains about 10-12 carbon atoms, and arylene is phenyl.

3. A fibrous article consisting essentially of a long-chain synthetic polyamide having recurring amide groups as an integral part of the main polymer chain, said poly-

5

10

15

amide having incorporated thereon an active amount of a compound having the formula



wherein X is an acid anion; Y is phenyl; R<sub>1</sub> is an alkyl of 1-4 carbon atoms; and R<sub>2</sub> is an alkyl which contains about 10-12 carbon atoms, and arylene is phenyl.

**References Cited by the Examiner**  
FOREIGN PATENTS

1,248,412 11/1960 France.

**OTHER REFERENCES**

Goldsmith: Chem. Abst., vol. 50, 1956, page 9023g.

JULIAN S. LEVITT, Primary Examiner.

MORRIS O. WOLK, IRVING MARCUS, Examiners.